

April 14, 1959

M. M. FREUNDLICH

2,882,502

WAVEGUIDE WINDOW

Filed April 19, 1954



FIG. 2



FIG. 1



FIG. 2a



FIG. 3



FIG. 3a

INVENTOR.  
MARTIN M. FREUNDLICH

BY

*Passaic, Edmund, Morton, Brown & Taylor*

ATTORNEYS

1

2,882,502

## WAVEGUIDE WINDOW

Martin M. Freundlich, Huntington Station, N.Y., assignor, by mesne assignments, to Cutler-Hammer, Inc., Milwaukee, Wis., a corporation of Delaware

Application April 19, 1954, Serial No. 423,893

11 Claims. (Cl. 333—98)

This invention relates to waveguide windows and a method of manufacture thereof, and is especially directed to the provision of a low-loss wideband window suitable for use over a substantial frequency range.

Waveguides are in common use for the transmission of ultra-high-frequency radio energy. For example, waveguides are in widespread use for the transmission of energy in the range of 3,000 megacycles per second (mc.) and are sometimes employed at lower frequencies. At still higher frequencies, such as 10,000 mc. and above, waveguides are used almost exclusively for transmission.

Usually the cross-sectional dimensions of the waveguide are selected to be smaller as the frequency of operation increases. The low frequency cutoff is determined largely by the dimensions selected, and the usefulness of a given waveguide is greatly impaired by spurious modes of transmission when the frequency exceeds some upper limit. Thus a waveguide of given cross-sectional dimensions is commonly employed only for a limited frequency range.

For practical reasons, the cross-sectional dimensions of waveguides have been considerably standardized in each frequency range. For example, in the region of 10,000 mc. a type of waveguide designated RG-52/U is often employed. This is a rectangular waveguide whose internal cross-sectional dimensions are approximately 0.90 x 0.40 inch and is employed to transmit frequencies in the range of about 8,200 to 12,400 mc. Other standard waveguides are available for other frequency ranges. Although waveguide of rectangular cross-section is most widely employed, circular waveguide is also used upon occasion, and the present invention is applicable to either type.

It is often desirable to place a window in a waveguide so as to permit maintaining a vacuum or pressure in one part of the waveguide with respect to another, or to exclude rain and moisture, etc. It is important that such a window have low losses so as to attenuate the transmitted energy as little as possible, and also to avoid setting up standing waves which might effect adversely the performance of equipment with which the waveguide is used. It is also highly desirable to have a window which will transmit energy over a wide frequency range with low attenuation and low standing wave ratio (SWR), preferably over the whole frequency range of the waveguide with which it is used, thus permitting use in applications where the transmission or reception of signals over a wide frequency range is required, and avoiding the need of producing and stocking a large number of narrow band windows for spot frequency applications.

There have been many proposals for constructing waveguide windows, and some have been used in practice. Most commercial windows have been of the resonant type, in which the area and thickness of the window and the design of the associated mounting are chosen so as to resonate at a certain frequency, thus

yielding a relatively low loss and low SWR at that frequency. While often satisfactory for a given application, such resonant structures inherently have a relatively narrow band, and the losses and standing wave ratio increase fairly rapidly outside of that band.

Glass has commonly been employed as the window material. However, even so-called "low-loss" glass in practical thicknesses introduces sufficient attenuation and dielectric discontinuity in a waveguide as to confine its usefulness largely to resonant type structures. It is also known that high-grade mica in thin sheets has very low losses at ultra-high frequencies, and some success has been attained with mica in windows of the resonant type.

It is a primary object of the present invention to provide a low-loss wideband waveguide window, and to this end mica is employed as the window material in a non-resonant structure. It is also an object of the invention to provide a window of this type which can be inserted readily in a waveguide. Other objects and advantages of the invention will in part be pointed out and in part be evident from the description given hereinafter.

In accordance with the invention, a thin sheet of mica is sealed between a pair of aligned metal frames having inside dimensions equal to the internal cross-sectional dimensions of the waveguide. The sheet of mica has planar dimensions greater than the inside dimensions of the frames and is sealed between the frames by a cementing material, preferably glass, which extends between the opposed surfaces of the frames so as to form a strong vacuum-tight seal. The cementing material advantageously extends substantially to, but not beyond, the inside edges of the frames. Particularly in the case of glass, this has been found to be of considerable importance in order to provide a strong seal and yet avoid losses and increased SWR. The thickness of the mica and cement layer is very small compared to a wavelength over the frequency range of the waveguide. As a result, it is found that when the window is soldered into a waveguide, the losses and SWR are very low over a wide range of frequencies.

The invention will be more fully understood by reference to the following detailed description thereof, taken in conjunction with the drawings, in which:

Fig. 1 is a perspective view of one specific window of the invention;

Fig. 2 is a cross-section taken along the line 2—2 of Fig. 1;

Fig. 2a is a detail illustrating an undesirable formation of the glass sealing layer;

Fig. 3 illustrates the window soldered in a section of waveguide; and

Fig. 3a is a view of one portion of the waveguide of Fig. 3, showing details of the flange recess.

Referring now to Fig. 1, a waveguide window is shown comprising a pair of aligned thin metal frames 10, 11, with a thin sheet of mica 12 sandwiched therebetween. The mica sheet is sealed between the metal frames by a cementing material, advantageously glass, which also joins the two metal frames 10, 11 so as to form a unitary structure.

The window of Fig. 1 is designed for use with a rectangular waveguide and the inner dimensions 13, 14 of the frames, that is, the dimensions of the window opening, are made equal to the internal cross-sectional dimensions of the waveguide with which it is to be employed.

Fig. 2 is a cross-section of the window of Fig. 1 and shows the metal frames 10, 11 sealed in alignment by a thin fused layer of glass 15. The mica sheet 12 has planar dimensions which are greater than the inside dimensions of the frames so that it overlaps the frames,

as shown at 12'. Thus, the glass layer 15 joins the mica sheet and the metal frames in a single unitary construction which is vacuum-tight.

Advantageously, as shown in Fig. 2, the planar dimensions of the mica sheet 12 are less than the outside dimensions of the frames, so that the fused layer of glass 15 extends between the opposed surfaces of the frames on both sides of the mica sheet and also around the outer edge thereof. Thus the mica sheet is firmly bonded to both metal frames, and the outer portions of the frames are directly bonded together by the fused glass. In effect, the mica sheet is embedded in the glass layer. The result is a very strong vacuum-tight joint.

The thickness of the mica sheet 12 and glass layer 15 is made very small compared to a wavelength over the frequency range of operation in a waveguide. Thus, when the window is inserted in a waveguide, the metal frames become part of the conducting waveguide wall and introduce no substantial discontinuity. The mica and glass layer does introduce a discontinuity, but the discontinuity is very short and consequently the losses and reflections caused thereby are very small.

It is desirable to select the metal of the frames and the glass so as to match the thermal coefficient of expansion of the mica as nearly as possible. Glass is preferred as the cementing material since it forms a strong permanent air-tight seal, and also will withstand ordinary soldering temperatures of, say, 250° C. or thereabouts. This is an important advantage, since soldering the metal frame into a waveguide insures good electrical contact to minimize the length of the discontinuity in the waveguide wall. However, for some purposes it may be found satisfactory to employ other cementing materials, such as plastic cements, etc.

In a particular window which has been used with success, the metal frames were punched out of Allegheny-Ludlum Alloy No. 4750 or Driver-Harris Alloy No. 52. These alloys are understood to contain approximately 50% nickel and 50% iron. The glass was Corning Type 7570, which is sometimes termed a "solder" glass. The window was specifically designed for use with waveguide type RG-52/U, mentioned above, and the internal dimensions 13 and 14 were 0.400 inch and 0.900 inch, respectively, to match the internal dimensions of the waveguide. The external dimensions of the window were .597 x 1.097 inches, and the thickness of each frame was .030 inch. A thin sheet of mica approximately 0.002 inch thick was employed, and the thickness of the glass layer 15 was approximately 0.006 inch, giving an overall thickness of the window of approximately 0.066 inch.

This window was found to have an average SWR of approximately 1.05 over the frequency range from 8200 to 12,400 mc. In a typical lot, the maximum standing wave ratio over this frequency range for the poorest window was 1.08. Taking a frequency near the middle of this range, 10,000 mc., the wavelength in air is 3 cm. (1.2 inches) and only slightly different in the waveguide. Thus the thickness of the mica-glass layer (0.006 inch) is very small compared to the wavelength.

In producing this window, the metal frames were first degreased, chemically cleaned and hydrogen-fired. The frames were then coated with a glass frit composed of the above-mentioned Corning glass mixed with water and heated in air to approximately 590° C. After cooling, the glass layer on the frames was ground to a thickness of approximately 0.003 inch.

The mica was then assembled between the frames and the assembly aligned in a jig. To facilitate handling and precise assembling, the mica was glued to the lower frame with a cellulose binder, and the upper frame then glued in place with the same binder. Small weights were placed on top of the assembly and the unit sealed together by baking at a temperature of about 600° C. for about 10-15 minutes to fuse the glass. The glueing

step is advantageous to secure proper alignment, and does not appear to affect adversely the final seal since the sealing temperature is sufficiently high to burn out the binder.

This process resulted in a strong vacuum-tight joint. However, the sealing procedure left a fillet of glass 15' at the inside edges of the metal frames of the nature illustrated in Fig. 2a. This glass fillet is highly undesirable since it considerably increases the SWR of the window. In rectangular waveguides of the type illustrated, it was found that if the fillet extended a few thousandths of an inch into the window area, on the long edges of the rectangle, there was a marked increase in SWR. The fillets on the narrow edges were not so objectionable due to the fact that the direction of the electrical field in rectangular waveguides is commonly perpendicular to the longer side. However, though of lesser importance, an excessive glass fillet on the narrow edges is undesirable. In the case of round waveguides, it is considered that the presence of the glass fillet at any point around the circumference of the window area is undesirable. If the glass layer recedes from the inner edges of the frames, the electrical properties of the window will not be affected materially, but the strength of the seal will be weakened and in many cases such weakening will be undesirable.

In order to eliminate the glass fillet, a glass is advantageously selected which, when contacted by an acid solution of suitable composition, is attacked by the acid so as to decompose the glass or destroy its vitreous nature, with resultant disintegration of the fillet. The fillet may then be removed by a small soft scraper, such as a pointed wooden stick.

The composition of the glass should be chosen with respect to that of the acid solution so that the glass can be disintegrated, as described, while at the same time the acid solution must be such as not to harm the metal frames. For the glass mentioned above, a first cleaning operation was effected by dipping the windows for two minutes in a bath made of 24 oz. sulphuric acid (commercial grade) in a gallon of water, at 90° C. This loosened the scale on the metal frames. The frames were then placed for two minutes at room temperature in a bath made as follows:

45 ½ pint sulphuric acid (commercial grade)  
½ pint hydrofluoric acid (commercial grade)  
8 oz. chromic acid  
Water to make one gallon.

This treatment removed the scale on the metal frames and also changed the glass of the fillet to a white powder which could be removed mechanically as described above. The depth to which the glass is attacked increases with duration of immersion, so that the duration can be selected with respect to the size of the glass fillet to be disintegrated and removed. Any glass remaining on the outside edge of the window may be ground off.

The frames were then silver-plated so as to insure making good contact with a waveguide. This was accomplished by cleaning the windows in a 50% solution by volume of nitric acid, silver-plating the windows, rinsing in running water, rinsing in acetone, and drying in a stream of air.

Referring now to Fig. 3, the window is shown inserted in a flange 16, 17 of a rectangular waveguide 18. The window made as described is capable of withstanding a considerable temperature, well above the temperature required for effective soldering. While the design of the flange is subject to considerable variation, depending upon the use contemplated, one design is shown in Fig. 3a. Here one section of waveguide 18 terminates in an outwardly extending flange 16 having a recess 21 whose dimensions accommodate the window.

One soldering technique which can be employed with this construction is to pre-tin the internal surfaces of

the recess 21 and apply a minimum amount of non-corrosive solder paste to the window frame edge and underside. The waveguide is held vertically, the window placed in the recess area, and the flange heated from the underside until the window drops in place and seats. Advantageously the depth of the recess 21 is substantially equal to the thickness of the frame of the window, so that the frame is flush with the surface of the flange when seated therein. Care should of course be taken to avoid any solder running onto the mica window area or in to adjacent portions of the waveguide opening. The matching section of the waveguide may be provided with a flat flange 17 which can thus be bolted to flange 16 in which the window is seated, or secured thereto in any suitable manner.

It will be apparent that many details of the specific embodiment described may be changed within the spirit and scope of the invention. Also, the numerical values given in the example described herein may be changed as required for a particular application, these values being given merely as an aid to the ready practice of the invention. The shape and overall dimensions will of course be altered for different sizes and shapes of waveguides. While the method of making the window described herein has been found satisfactory in practice, any other suitable method of making it may of course be employed if desired.

I claim:

1. A low-loss wideband window for an electromagnetic waveguide which consists of a pair of aligned metal frames of predetermined inside and outside dimensions, a thin sheet of mica having planar dimensions greater than said inside dimensions but less than the outside dimensions of said frames, said thin sheet of mica being substantially transparent to ultra-high-frequency electromagnetic energy, and a cementing layer sealing said mica sheet between said frames, said cementing layer extending substantially continuously around the border of each side of the mica sheet between the mica sheet and the opposed surface of the respective frame and substantially continuously outside the edges of the mica sheet between the opposed surfaces of the frames, said cementing layer firmly uniting said frames and firmly uniting each side of the mica sheet to the respective frame.

2. A low-loss wideband window for an electromagnetic waveguide which consists of a pair of aligned metal frames of predetermined inside and outside dimensions, a thin sheet of mica having planar dimensions greater than said inside dimensions but less than the outside dimensions of said frames, said thin sheet of mica being substantially transparent to ultra-high-frequency electromagnetic energy, and a cementing layer sealing said mica sheet between said frames, said cementing layer extending substantially continuously around the border of each side of the mica sheet between the mica sheet and the opposed surface of the respective frame and substantially continuously outside the edges of the mica sheet between the opposed surfaces of the frames, said cementing layer extending towards but not beyond the inside edges of the said frames and firmly uniting said frames and firmly uniting each side of the mica sheet to the respective frame.

3. A low-loss wideband window for an electromagnetic waveguide which comprises a pair of aligned metal frames of predetermined inside and outside dimensions, a sheet of mica having planar dimensions greater than said inside dimensions but less than the outside dimensions of said frames, said mica sheet being sealed between said frames by a fused glass layer joining both sides of the mica sheet near the edge thereof to the respectively opposed surfaces of the frames and joining together the opposed surfaces of the frames around the edge of the mica sheet, said glass layer extending substantially to but not beyond the inside edges of said frames.

4. A low-loss wideband window for an electromagnetic

waveguide which comprises a pair of aligned metal frames having rectangular window openings of predetermined dimensions, a sheet of mica having planar dimensions greater than said window opening dimensions but less than the outside dimensions of said frames, said mica sheet being sealed between said frames by a fused glass layer joining both sides of the mica sheet near the edge thereof to the respectively opposed surfaces of the frames and joining together the opposed surfaces of the frames around the edge of the mica sheet, said glass layer extending towards but not beyond the longer edges of said rectangular window openings of the frames.

5. A low-loss wideband window for insertion in an electromagnetic waveguide of predetermined inside cross-sectional dimensions which comprises a pair of aligned metal frames having inside dimensions equal to the inside cross-sectional dimensions of said waveguide, a sheet of mica having planar dimensions greater than said inside dimensions but less than the outside dimensions of said frames, said mica sheet being sealed between said frames by a cementing layer joining both sides of the mica sheet near the edge thereof to the respectively opposed surfaces of the frames and joining together the opposed surfaces of the frames around the edge of the mica sheet.

6. A low-loss wideband window for insertion in an electromagnetic waveguide of predetermined inside cross-sectional dimensions adapted to transmit ultra-high-frequency radio energy over a substantial frequency range which comprises a pair of aligned metal frames having inside dimensions equal to the inside cross-sectional dimensions of said waveguide, a sheet of mica having planar dimensions greater than said inside dimensions but less than the outside dimensions of said frames, said mica sheet being sealed between said frames by a fused glass layer joining both sides of the mica sheet near the edge thereof to the respectively opposed surfaces of the frames and joining together the opposed surfaces of the frames around the edge of the mica sheet, the thickness of the mica sheet and glass layer being very small compared to a wavelength over said frequency range.

7. A low-loss wideband window for insertion in an electromagnetic waveguide of predetermined inside cross-sectional dimensions adapted to transmit ultra-high-frequency radio energy over a substantial frequency range which comprises a pair of aligned metal frames having rectangular window openings of dimensions equal to the inside cross-sectional dimensions of said waveguide, a sheet of mica having planar dimensions greater than said window opening dimensions but less than the outside dimensions of said frames, said mica sheet being sealed between said frames by a fused glass layer joining both sides of the mica sheet near the edge thereof to the respectively opposed surfaces of the frames and joining together the opposed surfaces of the frame around the edge of the mica sheet, said glass layer extending substantially to but not beyond the longer edges of said rectangular window openings of the frames, the thickness of the mica sheet and glass layer being very small compared to a wavelength over said frequency range.

8. A low-loss wideband window for insertion in an electromagnetic waveguide of predetermined inside cross-sectional dimensions adapted to transmit ultra-high-frequency radio energy over a substantial frequency range which comprises a pair of aligned metal frames having inside dimensions equal to the inside cross-sectional dimensions of said waveguide, a sheet of mica having planar dimensions greater than said inside dimensions but less than the outside dimensions of said frames, said mica sheet being sealed between said frames by a fused glass layer joining both sides of the mica sheet near the edge thereof to the respectively opposed surfaces of the frames and joining together the opposed surfaces of the frames around the edge of the mica sheet, said glass layer

extending substantially to but not beyond the inside edges of said frames, the thickness of the mica sheet and glass layer being very small compared to a wavelength over said frequency range.

9. A method of making a low-loss window for an electromagnetic waveguide which comprises sealing a sheet of mica between a pair of aligned metal frames by a fused glass layer, heat and pressure being applied during said sealing whereby a fillet of glass is formed inside an inner edge of said frames, contacting said fillet with an acid solution selected to disintegrate the glass of said fillet, and removing said disintegrated fillet.

10. A method of making a low-loss window for an electromagnetic waveguide which comprises fusing a layer of glass to one side of each of a pair of metal frames, assembling a sheet of mica between said frames in contact with the glass layer, heating the assembly under pressure to fuse the glass layers and thereby form a sealing layer extending between the opposed surfaces of the frames on both sides of the mica sheet, said heating and pressure resulting in the formation of a fillet of glass inside an inner edge of said frames, contacting the assembly with an acid solution selected with respect to said glass to disintegrate said fillet, and removing said disintegrated fillet.

11. A method of making a low-loss window for an electromagnetic waveguide which comprises fusing a layer of glass to one side of each of a pair of metal frames, grinding the glass layer on each frame to a substantially uniform thickness, assembling a sheet of mica between said frames in contact with the glass layers, the planar dimensions of the mica sheet being greater than the inside dimensions of said frames but less than the outside dimensions thereof, heating the assembly under pressure to fuse the glass layers and thereby form a sealing layer extending between the opposed surfaces of the frames on both sides of the mica sheet and around the edge thereof, said heating and pressure resulting in the formation of a fillet of glass inside an inner edge of said frames, immersing the assembly in an acid solution selected with respect to said glass to disintegrate said fillet, and mechanically removing said disintegrated fillet.

References Cited in the file of this patent

UNITED STATES PATENTS

|              |          |               |
|--------------|----------|---------------|
| 2,198,769    | Goodale  | Apr. 30, 1940 |
| 2,453,645    | Tiley    | Nov. 9, 1948  |
| 2,556,881    | McArthur | June 12, 1951 |
| 25 2,636,926 | Wilson   | Apr. 28, 1953 |

UNITED STATES PATENT OFFICE  
CERTIFICATE OF CORRECTION

April 14, 1959

Patent No. 2,882,502

Martin M. Freundlich

It is hereby certified that error appears in the printed specification of the above numbered patent requiring correction and that the said Letters Patent should read as corrected below.

Column 6, line 55, for "frame" read -- frames --.

Signed and sealed this 28th day of July 1959.

(SEAL)

Attest:

KARL H. AXLINE

Attesting Officer

ROBERT C. WATSON  
Commissioner of Patents